

## UNITED STATES PATENT OFFICE.

CHARLES TOPPAN, OF SALEM, MASSACHUSETTS.

## BLEACHING COMPOUND.

SPECIFICATION forming part of Letters Patent No. 350,218, dated, October 5, 1886.

Application filed May 15, 1886. Serial No. 202,281. (No specimens.)

*To all whom it may concern:*

Be it known that I, CHARLES TOPPAN, of the city of Salem, in the county of Essex and State of Massachusetts, have invented an Improvement in Bleaching Compounds, of which the following is a specification.

The object of my invention is to produce a compound for bleaching cotton, linen, and other fabrics, composed of vegetable fibers or fibrous substances—such as raw cotton, flax, hemp, jute, wood pulp, &c.—containing vegetable coloring-matter in a convenient and very expeditious manner without reducing the strength of the finest fibers. I find by experiment that the detergent properties of my improved composition of matter is such that the fabrics, goods, and fibers bleached thereby are rendered very soft and pliable, and also more susceptible to receive and retain colors or dyes, particularly such as belong to the class of aniline colors.

In carrying out my invention I produce the new composition of matter about as follows: Take three parts, by measure, of expressed oil of mustard-seed; three parts, by measure, of melted paraffine; three parts, by measure, of caustic soda of 20° Baumé, and thoroughly mix the same, so as to form a saponaceous compound. Then take one part, by weight, of this compound and two parts, by weight, of pure tallow-soap and thoroughly mix the same together.

To prepare the bleaching solution, add one ounce of the above compound to each gallon of water contained in any suitable vessel, boiler, or keir; then add the same quantity, or one ounce, of sulphate of soda to each gallon of water; then add one fluid ounce of caustic soda, 20° Baumé, to each gallon of water; then heat the solution so as to dissolve the compound contained in the boiler; then immerse

the fabric, goods, or fibers in the hot solution and close the vessel; then boil the same sufficiently to bleach. The time required will vary according to the kind and quality of fabrics or 45 fibers being treated, and, as the compound will not injure the finest fibers, overboiling will not detrimentally affect the same.

I find by experiment that the above compound has an affinity for the coloring-matter 50 contained in cotton fabric, or raw cotton and similar vegetable fibers, and that it assimilates therewith and dissolves the same, so that it is very quickly and effectually freed and removed from the fiber of the cotton fabric or other 55 goods being bleached. With this compound the process of bleaching cotton or linen fabrics or similar vegetable fibers in a superior manner only requires from eight to ten hours, whereas the common process requires about 60 twenty-four hours to produce an inferior result. The tar-like coloring-matter contained in raw cotton or cotton fabric and similar textiles and the pyroligneous acid contained in wood pulp are so very fully and effectually 65 dissolved and freed from the fibers and removed by boiling the goods in this solution that they will remain perfectly white for a long time, and will not turn yellow when carried in stock, or when exposed to the rays of the sun. 70 An indefinite period, the bleaching is so thorough and permanent.

Having thus described my invention, what I claim is—

The above-described bleaching compound, 75 consisting of expressed oil of mustard-seed, paraffine, caustic soda, tallow-soap, sulphate of soda, and water, as set forth.

CHARLES TOPPAN.

Witnesses:

SYLVEONUS S. WALKER,

WILLIAM H. PARRY.